

1

2,917,394

SPARK PLUG INSULATORS CONTAINING  
STANNIC OXIDE

Harry G. Schurecht, Detroit, Mich., assignor to Champion Spark Plug Company, Toledo, Ohio, a corporation of Delaware

No Drawing. Application July 28, 1958  
Serial No. 751,175

6 Claims. (Cl. 106—46)

This invention relates to spark plug insulators containing stannic oxide, and, more particularly, to such insulators produced by firing particular compositions of oxide or oxide-forming materials including stannic oxide.

The use of tin oxide in making different refractory bodies has previously been suggested, for example, bodies suitable for use in contact with molten glass, and bodies having a high dielectric constant (in excess of one thousand in all instances) suitable for use as electro-mechanical devices such as piezo electric crystals.

Ceramic insulators having a dielectric constant greater than about 10 are completely unsuited for spark plug uses. Relatively high voltages are conducted interiorly through the electrode system of spark plug insulators. The air surrounding such insulators is ionized to a substantial extent by this electric current. The ionization of the air surrounding the insulator provides a potential path for spark discharge, for example from the metal connection at the top of an ordinary automotive spark plug to the grounded portion of the spark plug, or to a metallic component of an associated automobile engine. When the dielectric constant of the insulator is as high as about 10 such ionization occurs to an extent sufficient that discharge in this manner occurs to the exclusion of the desired discharge across the spark gap of the plug. Ceramic insulators can be produced from pure stannic oxide and also from mixtures of stannic oxide with minor amounts of fluxing ingredients. Such insulators, however, have properties which make them completely unsuited for use as spark plug ceramics. For example, a spark plug insulator is subjected to high temperatures in service, and must be effective at such high temperatures, as well as at low temperatures which are encountered in a cold engine and all intermediate temperatures. To be suited for spark plug use, a ceramic, in the form of a cylinder about  $\frac{1}{2}$ " in diameter and approximately  $\frac{1}{2}$ " in length must have an electrical resistance, at  $1350^{\circ}$  F. and at lower temperatures, of at least 1 megohm. Since it is a general characteristic of ceramic materials that their resistance decreases with increases in temperature, a particular ceramic can be shown to be suitable for spark plug use by determining that a cylinder thereof of the indicated size has an electrical resistance of at least 1 megohm at a temperature of  $1350^{\circ}$  F. or higher, or a given ceramic can be shown to be unsuited for spark plug use by a determination that such a cylinder thereof has a resistance of less than 1 megohm at a temperature of  $1350^{\circ}$  F. or lower. It has been determined that such a cylinder produced from pure stannic oxide or from a mixture of 96.5 parts of stannic oxide with 1.5 parts of whiting, 2.0 parts of talc and 1.5 parts of bentonite has a resistance of less than 0.1 megohm at a temperature of  $1000^{\circ}$  F. Neither of such insulators, therefore, is suited for spark plug use. This suggests that stannic oxide would be an undesirable constituent in a ceramic batch for use in the preparation of a spark plug insulator because stannic oxide in an appreciable amount would be expected to

2

have an undesirable effect upon electrical resistance, at least at elevated temperatures.

The terms "percent" and "parts" are used herein and in the appended claims to refer to percent and parts by weight, unless otherwise indicated.

The present invention is based upon the discovery that it is possible to produce sintered ceramic spark plug insulators by firing mixtures consisting essentially of alumina and stannic oxide, in certain proportions, and 10 that the resulting insulators not only have the dielectric properties requisite for spark plug use, but also have thermal conductivity characteristics which are at least equivalent to presently used spark plug ceramics, and are resistant to corrosion by compounds of lead and other chemicals which are present in the firing chambers of present-day internal combustion engines.

According to the invention, a sintered ceramic spark plug insulator is provided. Such an insulator is produced by firing a blend of refractory materials consisting 20 essentially of from about 19 parts to about 81 parts of  $\text{SnO}_2$  and from about 81 parts to about 19 parts of  $\text{Al}_2\text{O}_3$ . Insulators produced from such blends have the previously indicated properties, and limited amounts of other materials can be added to the blends, as will subsequently be discussed in more detail, without appreciably affecting such properties of insulators which are produced therefrom.

The suitability of various compositions consisting of stannic oxide and alumina, in proportions as set forth 30 above, for use in the manufacture of electrical insulators for spark plug purposes was demonstrated by preparing several insulators, and testing the properties of each. Representative examples of such compositions, and the properties of insulators produced therefrom, are given in 35 the following example, which, like the subsequent example, is to be construed as illustrative only, and not as limiting the invention.

## EXAMPLE 1

40 Several blends consisting of stannic oxide and alumina were wet milled to substantial uniformity (usually for 18 hours), and were then dried and mixed with 4 percent of paraffin wax, based upon the weight of dry ingredients, dissolved in carbon tetrachloride. The wax 45 was thoroughly mixed with the dry ingredients, and the carbon tetrachloride volatilized, leaving the wax uniformly dispersed throughout the composition. Test cylinders about  $\frac{1}{2}$ " in diameter and approximately  $\frac{1}{2}$ " in length were then pressed from each mixed composition, 50 using a total pressure of 10,000 pounds. The cylinders were then fired to Cone 31.

The bodies so prepared were tested to determine their suitability for use as spark plug insulators. The electrical resistance of the  $\frac{1}{2}$ " cylinders was determined at 55  $1200^{\circ}$  F. or  $1400^{\circ}$  F., and, in some instances, at  $1500^{\circ}$  F. As has been indicated above, a ceramic body having a resistance (when in the form of such a cylinder) of at least 1 megohm at  $1350^{\circ}$  F. or higher is considered satisfactory for spark plug purposes. In addition, an 60 insulator having a resistance of at least about 10 megohms at  $1200^{\circ}$  F. is considered satisfactory for spark plug purposes.

Another standard test was conducted to compare the thermal diffusivities of insulators produced from the 65 different compositions: The test involved placing a crystal of citric acid on one end of the sintered  $\frac{1}{2}$ " cylinder, and immersing the other end of the cylinder in a  $600^{\circ}$  F. metal bath to a depth of about  $\frac{1}{8}$ ". The number of seconds required for heat conducted through the insulator to melt the citric acid crystal, which melts at  $307.4^{\circ}$  F., is reported in the tables herein as "thermal diffusivity," 70 and is an inverse function of thermal conductivity. To

be at least comparable with presently used spark plug insulators in this respect, a ceramic insulator should have a thermal diffusivity, so measured, not greater than

herein, entries under the heading "Dye Test" are "Mat," which means matured; "U.F.," which means underfired, and "SUF," which means slightly underfired.

Table I

| Body No. | Composition in Parts           |                  | Electric Resistance (Megohms) |           |           | Thermal Diffusivity Time in Seconds | Dye Test |
|----------|--------------------------------|------------------|-------------------------------|-----------|-----------|-------------------------------------|----------|
|          | Al <sub>2</sub> O <sub>3</sub> | SnO <sub>2</sub> | 1,200° F.                     | 1,400° F. | 1,500° F. |                                     |          |
| 1        | 77.2                           | 19.3             | 80                            | 20        | 10.5      | 18.8                                | U.F.     |
| 2        | 57.9                           | 38.6             | 65                            | 20        | 10        | 19.5                                | U.F.     |
| 3        | 38.6                           | 57.9             | 10                            | -----     | -----     | 17.3                                | U.F.     |
| 4        | 19.3                           | 77.2             | 40                            | 12.8      | -----     | 20.9                                | U.F.     |

about 30 seconds. Ideally, a ceramic body should have a thermal diffusivity not greater than about 20 seconds.

A low thermal diffusivity time, or a high thermal conductivity, is an important characteristic of a spark plug insulator. In service, such an insulator is subjected to high temperatures in the firing chamber of an internal combustion engine. The insulator is heated to some temperature which depends, in the main, upon the mean effective firing chamber temperature, the thermal conductivity of the ceramic insulator and the design of the ceramic insulator and of the spark plug of which it constitutes a part. In general, high output present-day engines, when operated at or near full load, necessitate the use of spark plugs having thermal diffusivity times of 30 seconds or less in order to avoid heating of the ceramic insulator, in service, to a temperature sufficiently

20

25

30

## EXAMPLE 2

Table II, below, presents typical test results obtained with bodies produced from blends consisting essentially of Al<sub>2</sub>O<sub>3</sub> and SnO<sub>2</sub> in the previously indicated proportions. It will be observed from the results presented in Table II that substantial amounts of ZrO<sub>2</sub> can be employed in a blend used to produce an insulator according to the invention without adversely affecting the desirable characteristics of electrical resistance at elevated temperature and thermal diffusivity, and that limited amounts of whiting, talc and bentonite can be similarly added without adverse effect. All of the bodies reported in Table I, above, and in Table II, below, have been tested and found to be unexpectedly resistant to corrosion by lead and other compounds which are usually present in automotive and aviation fuels.

Table II

| Body No. | Composition in Parts           |                  |                  |         |       |           | Thermal Diffusivity Time in Seconds | Electric Resistance (Megohms) |           |           | Dye Test |
|----------|--------------------------------|------------------|------------------|---------|-------|-----------|-------------------------------------|-------------------------------|-----------|-----------|----------|
|          | Al <sub>2</sub> O <sub>3</sub> | SnO <sub>2</sub> | ZrO <sub>2</sub> | Whiting | Talc  | Bentonite |                                     | 1,200° F.                     | 1,400° F. | 1,500° F. |          |
| 5        | 57.9                           | 19.3             | 19.3             | -----   | ----- | -----     | 23.8                                | 48                            | 36        | 15        | SUF      |
| 6        | 57.9                           | 19.3             | 19.3             | 1.5     | 2.0   | 1.5       | 22.9                                | 100                           | 23        | -----     | Mat.     |
| 7        | 38.6                           | 38.6             | 19.3             | -----   | ----- | -----     | 29.4                                | 40                            | -----     | -----     | U.F.     |
| 8        | 19.3                           | 57.9             | 19.3             | -----   | ----- | -----     | 30.6                                | 30                            | -----     | -----     | U.F.     |
| 9        | 19.3                           | 38.6             | 38.6             | 1.5     | 2.0   | 1.5       | 27.8                                | 11.5                          | -----     | -----     | Mat.     |
| 10       | 77.2                           | 19.3             | -----            | 1.5     | 2.0   | 1.5       | 18.6                                | 100+                          | 100+      | 100+      | Mat.     |
| 11       | 57.9                           | 38.6             | -----            | 1.5     | 2.0   | 1.5       | 18.3                                | 100+                          | 50        | 38        | Mat.     |
| 12       | 38.6                           | 57.9             | -----            | 1.5     | 2.0   | 1.5       | 17.8                                | 45                            | 3.1       | -----     | SUF      |

high that it will cause premature ignition of a fuel-air mixture. Insulators having thermal diffusivity times of 20 seconds or less are ideal for use in such engines because more latitude is given a spark plug engineer in designing a plug which will operate satisfactorily without causing such premature ignition.

The insulators produced as described above were also subjected to tests to determine the adequacy of firing. The test involved application to each insulator of a dye solution, and visual examination of the so-treated insulator for evidence of dye absorption. Any insulator which absorbed dye was considered to be underfired, meaning that a higher firing temperature should be used, or that some fluxing material should be mixed with the composition to enable maturation under Cone 31 firing conditions. Insulators which did not absorb dye were either matured or overburned. These two states were distinguished by a specific gravity test, insulators having the highest specific gravity being properly matured and insulators which did not absorb the dye solution, but which had a lower specific gravity, being overfired.

Typical test results for bodies produced from blends consisting of alumina and stannic oxide, in the proportions indicated above, are presented in Table I, below. In Table I the composition of each blend is given, as well as the thermal diffusivity time, measured as discussed above, the electrical resistance at one or more of the indicated elevated temperatures, and, under the heading "Dye Test," the result of the above-described test for adequacy of a Cone 31 firing. In the tables

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

ticizer and binder, is preferably employed in producing an insulator according to the invention, and, most desirably, to the extent of from about 1 percent to about 2 percent, based upon the total weight of the blend, or ceramic batch. Both whiting and talc, as used in the blends or batches used in preparing the bodies reported in Table II, above, act as fluxes, tending to reduce the cone number designation of the firing required to effect maturation. Such a flux, or a different flux, is preferably employed in producing an insulator according to the invention, and, most desirably, to the extent of from about 1 percent to about 5 percent, based upon the total weight of the blend or ceramic batch. It is also preferred that the flux include an alkaline earth compound which, after firing, is in the form of the oxide, and most desired that it include, in addition to the alkaline earth compound, a magnesium silicate.

While reference has been made herein to stannic oxide, or  $\text{SnO}_2$ , as well as to alumina, or  $\text{Al}_2\text{O}_3$ , other tin oxides can be used in place of stannic oxide, or other tin compounds which revert to an oxide during firing, or compounds other than alumina which revert to alumina during firing can similarly be employed. Substantially the same properties result in the completed insulator. In addition, an entire insulator can be produced from a blend, as is disclosed in detail in the foregoing examples, or only a portion thereof can be produced from the blend, for example the firing tip, or the surface of the firing tip.

This is a continuation-in-part of application Serial No. 371,073, filed July 29, 1953, which was, in turn, a continuation-in-part of application Serial No. 69,409, filed January 5, 1949, both now abandoned.

It will be apparent that various changes and modifications can be made from the specific details set forth herein without departing from the spirit and scope of the attached claims.

What I claim is:

1. A ceramic spark plug insulator, at least the surface of which, at the firing end, is produced by sintering a blend consisting essentially of from about 19 parts to about 81 parts of  $\text{SnO}_2$ , and from about 81 parts to about 19 parts of  $\text{Al}_2\text{O}_3$ .

2. A ceramic spark plug insulator, at least the surface of which, at the firing end, is produced by sintering a blend consisting essentially of from about 19 parts to about 81 parts of  $\text{SnO}_2$ , and from about 81 parts to

about 19 parts of  $\text{Al}_2\text{O}_3$ , and including, in addition, based upon the total weight of the blend, from about 1 percent to about 5 percent of a flux.

3. A ceramic spark plug insulator, at least the surface of which, at the firing end, is produced by sintering a blend consisting essentially of from about 19 parts to about 81 parts of  $\text{SnO}_2$ , and from about 81 parts to about 19 parts of  $\text{Al}_2\text{O}_3$ , and including in addition, based upon the total weight of the blend, from about 1 percent to about 5 percent of a flux comprising an alkaline earth compound which, after firing, is in the oxide form.

4. A ceramic spark plug insulator, at least the surface of which, at the firing end, is produced by sintering a blend consisting essentially of from about 19 parts to about 81 parts of  $\text{SnO}_2$ , and from about 81 parts to about 19 parts of  $\text{Al}_2\text{O}_3$ , and including, in addition, based upon the total weight of the blend, from about 1 percent to about 5 percent of a flux comprising a magnesium silicate and an alkaline earth compound which, after firing, is in the oxide form.

5. A ceramic spark plug insulator, at least the surface of which, at the firing end, is produced by sintering a blend consisting essentially of from about 19 parts to about 81 parts of  $\text{SnO}_2$ , and from about 81 parts to about 19 parts of  $\text{Al}_2\text{O}_3$ , and including, in addition, based upon the total weight of the blend, from about 1 percent to about 5 percent of a flux comprising a magnesium silicate and an alkaline earth compound which, after firing, is in the oxide form, and from about 1 percent to about 2 percent of a plasticizer.

6. A ceramic spark plug insulator, at least the surface of which, at the firing end, is produced by sintering a blend consisting essentially of from about 19 parts to about 81 parts of  $\text{SnO}_2$ , and from about 81 parts to about 19 parts of  $\text{Al}_2\text{O}_3$ , and including, in addition, based upon the total weight of the blend, from about 1 percent to about 5 percent of a flux comprising a magnesium silicate and an alkaline earth compound which, after firing, is in the oxide form, and from 1 percent to 2 percent of bentonite.

#### References Cited in the file of this patent

#### UNITED STATES PATENTS

|    |           |           |               |
|----|-----------|-----------|---------------|
| 45 | 2,255,203 | Wiegand   | Sept. 9, 1941 |
|    | 2,413,441 | Feichter  | Dec. 31, 1946 |
|    | 2,577,369 | Schurecht | Dec. 4, 1951  |